

Dec. 1, 1936.

H. WATERMAN

2,062,543

ELECTROLYTE

Filed Oct. 22, 1935



INVENTOR

*Herbert Waterman*

BY

*Dean Fairbank, Hirsch Foster.*  
ATTORNEYS

## UNITED STATES PATENT OFFICE

2,062,543

## ELECTROLYTE

Herbert Waterman, Wantagh, N. Y., assignor to  
 Aerovox Corporation, Brooklyn, N. Y., a corpora-  
 tion of New York

Application October 22, 1935, Serial No. 46,070

9 Claims. (Cl. 175—315)

My present invention relates to electrolytic cells and while it has its preferred applicability to electrolytic condensers, it is also useful in electrical rectifiers, lightning arresters and similar structures, especially in such devices of the so-called dry type.

An object of the invention is to provide an electrolyte for the above use, composed of well-known ingredients approved for the purpose, but conditioned to produce substantial improvement in the resulting product, which in the case of the preferred application to condensers, insures substantial constancy of various electrical characteristics, including power factor, leakage and capacity, all of which maintain their optimum value throughout the life of the unit.

Another object is to provide an electrolyte agglomerate with the desired excess of solid ingredient, which yet presents no gritty structure but is and remains at all times extremely smooth and soft to admit of rapid incorporation into the absorbent separators of conventional condenser structures in the course of assembling them, as by a rolling operation, and which by virtue of its smoothness and softness remains in intimate contact with the electrode surfaces throughout the life of the condenser.

Another object is to provide a simple method, requiring simple apparatus for treating paste electrolytes of conventional character, with the result of imparting thereto the improved characteristics above noted.

As conducive to a clear understanding of the purpose of the invention, it is noted that commercial electrolytic condensers have been subject heretofore to more or less fortuitous variations in power factor, capacity and leakage in the course of use and especially under different conditions of use, and such variations have occurred regardless whether or not the unit was hermetically sealed. Efforts have been made to obviate these variations, but these have either failed entirely or involved the use of electrolytes or ingredients thereof, of prohibitive cost.

According to the present invention, these difficulties have been obviated by the simple expedient of homogenizing conventional paste electrolyte. The homogenization may be performed in any suitable apparatus, as, for instance, a conventional milk homogenizer, but it is preferred and found adequate for present purposes, simply to pass the electrolyte paste between a pair of heavy iron rollers, exerting a crushing pressure upon the crystals thereof, which results in a smooth soft creamy paste homogeneous

to the naked eye and even to a fairly strong magnifying glass.

Electrolytic condensers, especially of the dry type made according to conventional practice, as for instance, according to the teachings of Ruben Patent No. 1,710,073, when incorporating the homogeneous or comminuted paste of the present invention, in lieu of the same paste not so treated, show a surprising improvement in operation. In particular, the power factor of the freshly made condenser is improved in the order of 50 per cent, the leakage in the order of 5 to 10 per cent, the capacity per unit of area in the order of 10 per cent and moreover whatever electrical characteristics are present in the newly made condenser appear to be substantially preserved without appreciable change, even after the lapse of years whether on the shelf or in use.

While the theory is merely tentative, it is believed that the reason for the unexpected improvement in performance, as a result of the simple homogenization, comminution or crushing operation, is the stabilization of the physical structure of the paste thus treated. Electrolyte paste of conventional type, the solid ingredient of which comprises crystals generally precipitated from supersaturated hot solution, affords opportunity for growth of relatively large crystals about the initial nuclei precipitated. These larger crystals continue to grow as time goes on, the rate of growth decreasing as the temperature is reduced, but proceeding for months. This entails progressive change in the electrical characteristics of the condenser incorporating such electrolytes and more especially in the capacity and power factor thereof.

By the present invention, the homogenizing, comminution or crushing of the electrolyte paste after its crystals have reached fairly large size, reduces these crystals to minute size and since the paste aggregate is now largely of small solid crystals kept moist by the liquid carrier, with no great excess of such carrier, the aggregate is relatively stable physically and there is no marked opportunity for the crystals to grow as they might if the liquid carrier were in considerably greater volume relative to the volume of the crystals. Thus, the smooth creamy paste of the present invention remains stable, does not develop appreciable further crystallization within the condenser, and the original electrical characteristics for which the condenser is designed are maintained substantially constant throughout the useful life of the unit.

The electrolyte of the present invention, while

advantageously used with anodes made of smooth plates or foils, has particular utility with foils, the superficial area of which has been increased as by an etching process. The smooth electrolyte 5 paste with its minute crystals is thus permitted more effectively to enter the minute pits or depressions of etched foil, rendering the entire surface thereof effective from the standpoint of capacity, where the larger crystals of a coarser paste 10 might bridge across such pits or depressions and prevent adequate contact by the liquid ingredient of the electrolyte, with consequent impairment of power factor and loss of effective capacity.

Where paste electrolyte is employed that has 15 not been subjected to the mechanical comminution, homogenization or crushing operation, it is difficult to roll the condensers, for in rapidly stiffening and crystallizing, the paste becomes relatively hard and difficult to apply. At best, the 20 application of such a paste is uncertain.

By the treatment of the electrolyte as set forth, and the resultant smoothness and softness of the aggregate, it is feasible to pass the gauze or paper interlay through the paste electrolyte to become 25 impregnated therewith in the course of enrolling the gauze or paper with the foil.

In the single figure of the drawings, there is shown in purely diagrammatic form, an installation for the preparation of the electrolyte and the 30 incorporation thereof in the condenser.

The electrolyte paste is fed through the outlet nozzle 11 of a hopper 10 to the roller press or mill made up of contacting rollers 12 and 13 whence the comminuted soft paste is fed along a chute 35 14 into a tank 15 thermostatically kept at a temperature preferably in the neighborhood of 180 degrees F. The gauze, paper or other porous interlay 16 is fed from a roll 17 through the paste 18 in the tank 15, excess being removed by scrapers 19 and the interlay impregnated with the paste 40 is passed on to form the condenser roll R by sandwiching between two layers of foil 20 and 21 fed from corresponding rolls 22 and 23 respectively. Since a second interlay is needed in all structures 45 of the type under consideration to prevent direct contact between the upper surface of foil 20 as shown in the drawing, and the lower surface of foil 21, the roll for such interlay is shown at 17' and the material is fed through the electrolyte in 50 the same manner as in the case of roll 17, corresponding elements for feeding the second interlay having the same reference numerals primed as those for the first. It is understood that at least one of the foils 21 is pre-formed with the di-electric film, the other foil 20 being unformed in the 55 case of a polarized condenser while for an alternating current motor starting condenser, both of the foils would be pre-formed.

While the invention is not limited to the use of 60 any particular composition of paste electrolyte or mode of compounding the same, it has specific utility with an electrolyte made up of polyhydric alcohol such as glycerin or ethylene glycol and alkali borate, ordinarily ammonium borate. The 65 alkali borate, such as ammonium borate, may be introduced as such, preferably as ammonium pentaborate or the equivalent proportions of boric acid and ammonium hydroxide might be used. The proportions are such as to include the excess 70 of salt to produce the paste. The ingredients may be combined in any manner adequate to produce the paste, but preferably according to the teachings of Georgiev Patent No. 1,815,768, by driving off water until a definite predetermined boiling point has been attained, which boiling point will 75

vary somewhat with the voltage of use. Where ethylene glycol is used as the polyhydric alcohol, in combination with the ammonium borate and boric acid, the boiling point for a 500 volt condenser would be in the neighborhood of 130 degrees C. or 266 degrees F. which electrolyte is also suitable for lower voltages, although a boiling point somewhat lower, say 120 degrees C. or 250 degrees F. will result in a better power factor for lower voltage ranges in the order of 100 volts. 10 In the illustrative example the specific proportions may be 20 parts by weight of glycol, 20 parts by weight of ammonium pentaborate, and 10 parts by weight of boric acid.

In practice, the electrolyte in the gauze or paper 15 16, rapidly cools to room temperature, after leaving the tank 15, without marked change in the crystalline structure thereafter. However, the mass of electrolyte remaining in the tank at 180 degrees F. for prolonged periods, say for 24 hours, 20 will show evidence of increase in the size of crystals. It is, therefore, desirable from time to time to pass the contents of the tank 15 through the rolling mill 12, 13 for again reducing the size of 25 the crystals.

It will thus be seen that there is herein described electrolyte and method for preparing the same, in which the several features of this invention are embodied, and which method in its 30 action attains the various objects of the invention and is well suited to meet the requirements of practical use.

As many changes could be made in the above 35 method, and many apparently widely different embodiments of this invention could be made without departing from the scope thereof, it is intended that all matter contained in the above 40 description or shown in the accompanying drawing shall be interpreted as illustrative and not in a limiting sense.

Having thus described my invention, what I 45 claim as new and desire to secure by Letters Patent is:

1. The method of preparing a paste electrolyte 45 of the type comprising crystals moist with liquid having salt dissolved therein and useful in electrolytic cells, which consists in mechanically comminuting the crystalline structure thereof to render the paste relatively smooth and to inhibit the regrowth of crystals.

2. The method of preparing an electrolyte for 50 electrolytic cells, which consists in preparing a hot supersaturated solution of salts, permitting the material to crystallize and then mechanically 55 comminuting the crystal structure in the electrolyte to produce a relatively smooth and homogeneous product, in which regrowth of crystals is inhibited.

3. The method of preparing an electrolyte for 60 electrolytic cells, which consists in admixing polyhydric alcohol and alkali borate in proportions to produce a paste comprising crystals moist with liquid having salt dissolved therein and subjecting the paste to a mechanical crushing action 65 to comminute the crystals.

4. The method of preparing an electrolyte of 70 ingredients including glycerin, ammonia and boric acid, with the salt in proportion in excess of what will combine with or dissolve in the liquid portion; which method consists in cooking the ingredients to produce a hot supersaturated solution of substantially predetermined boiling point, permitting the mass to cool and crystallize 75

into an agglomerate and then substantially homogenizing the product.

5. The method of preparing an electrolyte of ingredients including polyhydric alcohol of the group comprising glycerin and ethylene glycol, ammonia and boric acid, with the salt in proportions in excess of what will combine with or dissolve in the liquid portion, which method consists in cooking the ingredients to produce a hot supersaturated solution of substantially predetermined boiling point, permitting the mass to cool and crystallize into a paste and then subjecting the paste to a mechanical crushing action to comminute the crystals.
15. 6. The method of preparing an electrolyte of ingredients including ethylene glycol, ammonia and boric acid, with the salt in proportions in excess of what will combine with or dissolve in the liquid portion, which method consists in cooking the ingredients to produce a hot supersaturated solution of substantially predetermined boiling point, permitting the mass to cool and crystallize into a paste and then feeding the paste between rollers to crush or comminute the individual crystals.
7. An electrolyte for electrolytic cells made of ingredients including polyhydric alcohol, and ammonium borate, the physical structure of said electrolyte comprising a smooth mass made up of a multiplicity of minute crystals of one or

more of the ingredients and a liquid carrier substantially moistening said crystals and without free excess.

8. The method of treating an electrolyte agglomerate comprising crystals moist with liquid having salt dissolved therein and incorporating it into an electrolytic cell, which consists in subjecting said agglomerate mechanically to comminution of its solid ingredient, maintaining the comminuted electrolyte in heated condition and before substantial crystal regrowth has occurred passing absorbent interlay therethrough and then incorporating the thus impregnated interlay with the electrodes in a condenser structure.

9. The method of treating paste electrolyte comprising crystals moist with liquid having salt dissolved therein and incorporating it in an electrolytic cell, which consists in subjecting the paste electrolyte mechanically to comminution of its crystalline structure, maintaining the comminuted electrolyte in heated condition, while passing absorbent interlay therethrough, and then incorporating the thus impregnated interlay with the electrodes in a condenser structure, and preventing excessive growth of crystals in the supply of previously comminuted electrolyte by subjecting said electrolyte to further mechanical comminuting action.

HERBERT WATERMAN. 30